

Patented May 8, 1928.

1,668,917

# UNITED STATES PATENT OFFICE.

CARL PIERCE LEWIS, OF BURLINGAME, CALIFORNIA, ASSIGNOR TO MINERALS SEPARATION NORTH AMERICAN CORPORATION, OF NEW YORK, N. Y., A CORPORATION OF MARYLAND.

## FROTH-FLOTATION CONCENTRATION OF ORES.

No Drawing.

Application filed July 28, 1925. Serial No. 46,860.

This invention relates to the froth-flotation concentration of ores, and is herein illustrated as applied to the concentration of what are known to miners and concentrator mill men as oxidized ores. Such ores may be true carbonates, but are often partly or largely sulphates, hydroxides, oxides and analogous compounds and usually are quite complex and contain a relatively large amount of primary gangue slimes, viz., slimes present in the ore in its natural state as distinguished from slimes produced by grinding the ore. The invention is well adapted for the concentration of such ores in which the values are present as carbonates or as basic hydroxides as well as ores in which the presence of primary gangue slimes makes ordinary flotation treatment ineffective.

According to this invention the concentration may often be effected without the use of any of the sulphidizing agents, so-called. Not only does this eliminate an expensive operation, but it also, in treating some silver-bearing ores, avoids the falling off of silver recovery which almost invariably follows when the step of sulphidization is introduced into the process of concentration.

It has been found that when certain carbonate ores are concentrated by froth-flotation in the presence of an organic sulphhydric compound such as a xanthate the tailings are cleaner and the concentrate is richer if a small proportion of a soluble silicate, such as sodium silicate, is present in the pulp. Under these conditions, although soluble silicates have normally no substantially beneficial effect on oxidized minerals, the recovery of both lead and silver from a lead carbonate ore is often substantially better than has hitherto been obtained. Under the same conditions the recovery of copper from an oxidized ore containing a relatively large amount of primary gangue slimes may approach the recovery of sulphide copper from easily floatable ores.

A pulp of a lead carbonate silver-bearing ore from the Blacksmith Tunnel of Senator mine, Arizona, adjacent to the Schuylkill mine, in which the lead was in the form of carbonate and sulphate, but which contained practically no lead sulphide, was agitated fifteen minutes in a subaeration machine

with Barrett #2 creosote 1. pound, American Tar and Turpentine Company's #11 destructively distilled pine oil 0.15 pound, potassium xanthate mother liquor (about half ethyl alcohol, and most of the remainder potassium xanthate) 0.4 pound, and sodium silicate 1. pound, all per ton of ore. The concentrate thus obtained was reagitated five minutes to yield a finished concentrate and a middling. The results are shown in the following table:

|            | Per cent weight | Per cent assays |      | Per cent recoveries |      |
|------------|-----------------|-----------------|------|---------------------|------|
|            |                 | Ag. (oz.)       | Pb.  | Ag.                 | Pb.  |
| Heads..... | 100.            | 22.0            | 5.4  |                     |      |
| Conc.....  | 14.6            | 128.1           | 26.4 | 85.1                | 71.1 |
| Midd.....  | 26.1            | 6.0             | 4.0  | 7.1                 | 19.2 |
| Tails..... | 59.3            | 2.9             | 0.9  | 7.8                 | 9.2  |

Other tests indicated that the mother liquor and the xanthate itself were substantial equivalents for use in this process.

Other tests of the same ore from other parts of the mine, varying considerably in composition, yielded comparable results. Tests of the tailings from these showed that the lead carbonate had almost completely passed into the concentrate.

Another silver-bearing lead-carbonate ore from the Eureka Nevada district, also almost free from lead sulphide, and containing the lead as carbonate and sulphate, was agitated for fifteen minutes in a subaeration machine with xanthate mother liquor 0.8 pound, sodium silicate 1.3 pounds, and American Tar and Turpentine Co's. crude pine oil 0.4 pound to yield a rougher concentrate. This concentrate was reagitated with added water to yield a finished concentrate and a middling. The results are shown in the following table:

|            | Per cent weight | Per cent assays |      | Per cent recoveries |      |
|------------|-----------------|-----------------|------|---------------------|------|
|            |                 | Ag. (oz.)       | Pb.  | Ag.                 | Pb.  |
| Heads..... | 100.            | 3.95            | 11.8 |                     |      |
| Conc.....  | 18.2            | 11.7            | 45.6 | 54.0                | 70.4 |
| Midd.....  | 27.1            | 2.7             | 7.2  | 25.3                | 16.6 |
| Tails..... | 54.7            | 1.5             | 2.8  | 20.7                | 13.0 |

Tests of the tailings showed that the lead carbonate had almost completely passed into the concentrate.

In some cases it may be advisable to col-

lect the froth-concentrate in two stages, only adding the soluble silicate after the values recoverable without it have been floated in the form of a froth and separated. Sometimes the addition of a soluble sulphide has been found advantageous, as in the following test of Silver Dyke mine ore of Montana. The ore was ground and then reground with potassium xanthate 0.3 pound, pine oil 0.5 10 pound, both per ton of ore. Water was then added and the pulp agitated for fifteen minutes in a subaeration machine, with removal of the froth, there was then added sodium silicate 0.8 pound, and sodium sulphide 3.5 pounds, both per ton of ore and the further froth formed was removed. The 15 collected froths were then reagitated for five minutes to form a finished concentrate and a middling. The results are shown in the following table:

| 25         | Per cent weight | Assays    |      |      | Recoveries |     |      | 85 |  |
|------------|-----------------|-----------|------|------|------------|-----|------|----|--|
|            |                 | Ag. (oz.) | Cu.  |      | Ag.        | Cu. |      |    |  |
|            |                 |           | Cu.  | Pb.  |            | Cu. | Pb.  |    |  |
| Heads..... | 100.            | 5.26      | 1.10 | 2.26 | 68.8       | 49. | 51.3 |    |  |
| Conc.....  | 6.              | 58.6      | 8.96 | 19.4 |            |     |      |    |  |
| Midd.....  | 19.8            | 4.0       | 1.0  | 1.8  | 15.0       | 18. | 15.9 |    |  |
| Tails..... | 74.2            | 1.03      | 0.48 | 1.0  | 18.2       | 33. | 32.8 |    |  |

30

The procedure of adding the soluble silicate after the separation of such values as are floatable without it, is especially valuable in concentrating certain copper ores, such as those containing both chalcocite and oxide, or acid-soluble copper. The following example illustrates the results obtainable.

40 A pulp of Ray Consolidated ore was agitated five minutes in a subaeration machine with potassium xanthate 0.2 pound, and pine oil 0.15 pound, both per ton of ore, and the froth removed to form a first concentrate. The remainder of the pulp was agitated ten minutes with the further addition of sodium silicate 0.6 pound, and pine oil 0.25 pound, both per ton of ore, and the froth removed to form a second concentrate. The results are shown in the following table from which it will be seen that the major portion of the oxide or acid-soluble copper was recovered in the second concentrate.

| 55           | Per cent weight | Assays |         | Recoveries |         | 120 |
|--------------|-----------------|--------|---------|------------|---------|-----|
|              |                 | Cu.    | Ox. Cu. | Cu.        | Ox. Cu. |     |
| Heads.....   | 100.            | 1.08   | 0.16    | 55.6       | 8.7     |     |
| Conc. 1..... | 2.7             | 22.24  | 0.52    |            |         |     |
| Conc. 2..... | 4.4             | 5.44   | 1.68    | 22.1       | 45.6    |     |
| Tails.....   | 92.9            | .26    | .08     | 22.3       | 45.7    |     |

60 In these analyses the oxide copper is separately given but is also included in the general copper analyses, which show the total

percentages of copper present in the heads and products.

Where there is no advantage in separating a first froth before adding the soluble silicate, excellent results have been obtained by the procedure of agitating copper ores in the presence of all the mineral-frothing and other flotation agents, including the sodium silicate. The following example illustrates the results obtainable.

75 A pulp of a highly oxidized ore from K. C. Y. Copper Co. mine, Chloride, Arizona, with a schist gangue, was agitated in a subaeration machine for fifteen minutes with potassium xanthate, 0.9 pound, sodium silicate, 1.5 pounds, and crude pine oil, 0.6 pound, all per ton of ore. The results are shown in the following table:

|            | Per cent weight | Assays |         | Recoveries |         | 90 |
|------------|-----------------|--------|---------|------------|---------|----|
|            |                 | Cu.    | Ox. Cu. | Cu.        | Ox. Cu. |    |
| Heads..... | 100.0           | 2.0    | 1.81    |            |         |    |
| Conc.....  | 20.6            | 8.08   | 7.44    | 81.0       | 84.5    |    |
| Tails..... | 79.4            | .48    | .36     | 19.0       | 15.5    |    |

The general copper percentages include the oxide copper in these analyses as in those next above given.

95 This test yielded a better result than any obtainable from the same ore when using a sulphidizing agent. Upon retreating a similar concentrate obtained in another test of this ore, the finished concentrates assayed 16.15% copper, of which 13.22% was present as oxide or acid-soluble copper.

100 Having thus described certain applications of the invention what is claimed is:

1. The process of concentrating oxidized ores which consists in agitating a pulp of the ore with a xanthate and a soluble silicate under such conditions that a mineral-bearing froth is produced, and separating the froth.

105 2. The process of concentrating oxidized ores which consists in agitating a pulp of the ore with an organic sulphhydric compound in the presence of a soluble silicate facilitating the recovery of oxidized metalliferous mineral and a mineral-frothing agent to form a mineral-bearing froth, and separating the froth.

110 3. The process of concentrating oxidized ores which consists in agitating a pulp of the ore with a xanthate and a mineral-frothing agent and a soluble silicate to form a mineral-bearing froth, and separating the froth.

115 4. The process of concentrating an ore containing a substantial amount of primary gangue slime which consists in agitating a pulp of the ore with a xanthate and a soluble silicate under such conditions that a mineral-bearing froth is produced relatively free from primary gangue slimes, and separating the froth.

5. The process of concentrating an ore containing a substantial amount of primary gangue slimes which consists in agitating a pulp of the ore with an organic sulphhydric compound and a mineral-frothing agent in the presence of a soluble silicate facilitating the recovery of oxidized metalliferous mineral to form a mineral-bearing froth relatively free from primary gangue slimes, and 10 separating the froth.

6. The process of concentrating an ore containing a substantial amount of primary gangue slime which consists in agitating a pulp of the ore with a xanthate and a mineral-frothing agent and a soluble silicate to 15 form a mineral-bearing froth, and separating the froth.

7. The process of concentrating carbonate ores which consists in agitating a pulp

of the ore with a xanthate and a mineral-frothing agent so as to produce a mineral-bearing froth, separating the froth, further agitating the pulp with further addition of silicate of soda so as to produce a second mineral-bearing froth, and separating the 20 second froth.

8. The process of concentrating oxidized ores which consists in agitating a pulp of the ore with an organic sulphhydric compound and a mineral-frothing agent so as to 30 produce a mineral-bearing froth, separating the froth, further agitating the pulp with the addition of a soluble silicate so as to produce a second mineral-bearing froth, and separating the second froth. 35

In testimony whereof, I have affixed my signature to this specification.

CARL PIERCE LEWIS.